

## 1

2,950,235

## ACID COPPER ELECTROPLATING BATHS

Wennemar Strauss and Wolf-Dieter Willmund, Dusseldorf-Holthausen, Germany, assignors to Dehydag, Deutsche Hydrierwerke G.m.b.H., Dusseldorf, Germany, a corporation of Germany

No Drawing. Filed Dec. 4, 1958, Ser. No. 778,075

Claims priority, application Germany Dec. 17, 1957

8 Claims. (Cl. 204—52)

This invention relates to acid copper plating baths containing organic compounds as brightening additives. It more specifically relates to an electroplating method and the baths therefore which eliminate anode sludge by the addition of new additives to the acid copper plating bath.

Acid copper electroplating baths which are usually operated with organic electroplating additives often have the disadvantage that they form a considerable amount of anode sludge. This sludge consists of finely dispersed, probably oxidized copper particles which also reach the objects to be copper plated by electrophoresis and thereby considerably reduce the quality of the copper electro-deposits. The typical blue color of the acid copper baths is discolored green through the presence of these fine particles.

It has been attempted to avoid the formation of the anode sludge by using specially alloyed (phosphorus-containing) copper anodes. It has further been attempted to eliminate the presence of impurities by constantly filtering the baths through filter aggregates and/or surrounding the anodes with filter bags. Despite these measures it is unavoidable that small amounts of colloidal impurities remain in the copper bath.

It has also been proposed to eliminate the bath impurities by blowing air therethrough or by adding oxidizing agents, such as hydrogen peroxide. By blowing air through the bath the impurities are oxidized into copper-II-compounds which are again transformed into copper sulfate by the sulfuric acid in the bath, but this method is not recommended in most cases, especially if the copper baths are operated with wetting agents, because of the strong foam formation.

The addition of hydrogen peroxide leads to the destruction of the impurities within a short time, but this method has the disadvantage that it causes the copper electroplates to become brittle and that the usable current density range is greatly reduced. For this reason, if the copper electroplating bath is regenerated with hydrogen peroxide the bath must be taken out of operation for an extended period of time until all of the hydrogen peroxide has decomposed.

All of the measures described above make the operation of acid copper electroplating baths considerably more difficult and require additional work or additional apparatus. Moreover, in these methods, it was unavoidable that some sludge particles deposited with the electro-deposit.

It is an object of this invention to prevent anode sludge formation in acid copper plating baths.

Another object is to provide an electroplating bath free from colloidal impurities.

Yet another object is to provide a method and bath for acid copper plating wherein auxiliary measures to maintain purity of the bath such as filtering, oxidation, special anodes, etc. are unnecessary.

Another object is to provide a method for obtaining a high quality copper deposit free from impurities in an acid copper plating bath such as anode sludge particles.

Another object is to provide an additive compound for acid copper plating baths which maintains the bath in a highly pure state.

## 2

We have now found that all of these disadvantages of the prior art methods can be avoided and the objects of our invention achieved by adding to the acid copper electroplating baths organic sulfonic acids containing at least one azido (triazo) group in the molecule or salts of such compounds. The addition of these compounds has the effect that the baths remain deep blue in color and clear and do not form a sludge throughout their entire period of operativeness, even if they are operated at high loads, whereas baths which are operated without these additives turn green after 2-4 a.h./liter acid and after some additional time begin to produce anode sludge.

At the same time, the novel products also produce a certain brightening effect. The brightness can be improved by further adding known brighteners to the baths. Examples of brighteners which may be used are: thiourea and its derivatives, N-mono- and di-substituted dithiocarbamic acid alkyl esters- $\omega$ -sulfonic acids or their salts, 1,3,5-triazine-2,4,6-tris-(mercaptoalkane-sulfonic acids). Brighteners of these types are disclosed in French Patent 1,097,123, Belgian Patents 543,413 and 540,564 and in our copending application Serial No. 618,183, now United States Patent No. 2,849,352. Furthermore, the customary wetting agents and/or known compounds which improve the ductility of the electroplates may be added to the baths.

The organic sulfonic acids containing azido groups have the following general structural formula:



wherein R is a lower saturated aliphatic hydrocarbon radical or an aromatic hydrocarbon radical, Z is an azido group and n is a whole number of at least one.

Examples of organic sulfonic acids having at least one azido group in the molecule are the following:

- 3-azido-propane-sulfonic acid-1
- 4-azido-butane-sulfonic acid-1
- 1-azido-1,1-dimethyl-propane-sulfonic acid-3
- 3-azido-2-hydroxy-propane-sulfonic acid-1
- 2-azido-3-halo-propane-sulfonic acid-1
- 2,3-diazido-propane-sulfonic acid-1
- 2,3-diazido-butane-sulfonic acid-1
- 8-azido-naphthalene-sulfonic acid-1
- 4-azido-benzene-sulfonic acid
- 2-(azido-methyl)-benzene-sulfonic acid

These compounds may be produced in accordance with known processes, for example by reacting sultones, such as propane sultone, tolylsulfone and 1,8-naphthylsulfone, with hydrazoic acid or its salts (azides) or by reacting hydrazoic acid or its salts with halogen-substituted organic sulfonic acids.

The acids are customarily used in the form of their water-soluble salts. Inorganic or organic bases, such as the alkali metals, ammonia, dialkylamines or dialkanolamines, may be used as salt forming components.

The compounds according to the present invention are added to the acid copper electroplating baths in amounts of 0.05-4.5 gm./liter, preferably of 0.2-0.8 gm./liter. The operating temperatures of such baths, which are usually operated within a current density range of 0 to 12.5 amp./dm.<sup>2</sup>, may vary within wide limits up to about 60° C.

The following examples are set forth to enable persons skilled in the art to better understand and practice the invention. It will be understood that there is no intention of limiting the invention to these examples.

## Examples

- 70 An acid copper electroplating bath containing 220 gm./liter CuSO<sub>4</sub>·5H<sub>2</sub>O, 60 gm./liter H<sub>2</sub>SO<sub>4</sub>, 0.05 gm./liter N,N-diethyl-dithiocarbamic acid ethyl ester- $\omega$ -sodium sul-

fonate as a brightener, 0.25 gm./liter 1,3-bis-(dibutylamino)-propanol-2 as a ductility-improving agent, and 1 gm./liter of the reaction product of dodecyl alcohol and 8 mols ethylene oxide as a wetting agent, was modified with 0.5 gm./liter  $\omega$ -azido-propane-sodium sulfonate. Full bright copper electroplates were obtained upon electroplating objects made of brass, bronze, iron or steel therein. The bath can be operated within a temperature range of about 15° to about 50° C. The useable current densities at 15° C. lie between 0 and 4.5 amp./dm.<sup>2</sup>, at 25° C. between 0 and 8 amp./dm.<sup>2</sup>, and at 50° C. between 1 and 12.5 amp./dm.<sup>2</sup>. The copper electroplating bath did not discolor and retained its blue color, even after prolonged periods of operation. Sludge formation at the copper anodes did not occur. Neither recycling pumps, filters, or anode bags were required. A sludge free deposit of copper was obtained.

Without the addition of  $\omega$ -azido-propane-sodium sulfonate the bath must be continuously recycled and filtered. Despite filtration, a certain amount of reduction in the brightness may occur, which is undesirable.

In place of  $\omega$ -azido-propane-sodium sulfonate the following compounds were used according to the examples above in amounts of 0.2 to 0.8 gm./liter with comparable results:

3-azido-2-hydroxy-propane-sulfonic acid-1  
2-azido-3-halo-propane-sulfonic acid-1  
2,3-diazido-propane-sulfonic acid-1  
3-azido-butane-sulfonic acid-1  
8-azido-naphthalene-sulfonic acid-1  
4-azido-benzene-sulfonic acid or their water-soluble salts.

While we have disclosed certain specific embodiments of our invention, we wish it to be understood that these are not intended to be limitative, and that various changes and modifications may be made without departing from the spirit of our invention or the scope of the appended claims.

We claim:

1. An acid copper electroplating bath for producing copper electrodeposits of high quality free from anode sludge, comprising an aqueous acid solution of a copper salt and a compound selected from the group consisting of compounds having the following general structural formula:



and water soluble salts thereof, wherein R is a radical selected from the group consisting of lower aliphatic saturated hydrocarbon and aromatic hydrocarbon radicals, Z is an azido group and n is a whole number of at least one, said compound being added in an amount sufficient to prevent sludge formation.

2. An acid copper electroplating bath for producing copper electrodeposits of high quality free from anode sludge comprising an aqueous acid solution of a copper salt, an organic brightening agent in an amount sufficient to effect brightening, and a compound selected from the group consisting of compounds having the following general structural formula:



and water soluble salts thereof, wherein R is a radical selected from the group consisting of lower aliphatic saturated hydrocarbon and aromatic hydrocarbon radicals, Z is an azido group and n is a whole number of at least one, said compound being added in an amount sufficient to prevent sludge formation.

3. An acid copper electroplating bath for producing copper electrodeposits of high quality free from anode sludge comprising an aqueous acid solution of a copper salt; a brightening agent selected from the group consisting of N-mono- and di-substituted dithiocarbamic acid alkyl ester- $\omega$ -sulfonic acids and their salts, and 1,3,5-triazine-2,4,6-tris-(mercapto-alkane-sulfonic acids), the amount of said brightening agent being sufficient to effect said brightening; and a compound selected from the group consisting of compounds having the following general structural formula:

cient to effect said brightening; and a compound selected from the group consisting of compounds having the following general structural formula:



and water soluble salts thereof, wherein R is a radical selected from the group consisting of lower aliphatic saturated hydrocarbons and aromatic hydrocarbon radicals, Z is an azido group and n is a whole number of at least one, said compound being added in an amount sufficient to prevent sludge formation.

4. An acid copper electroplating bath for producing copper electrodeposits of high quality free from anode sludge comprising an aqueous acid solution of copper sulfate, at least 0.01 gm./liter of N,N-diethyl-dithiocarbamic acid ethyl ester- $\omega$ -sodium sulfonate and 0.05 to 4.5 gm./liter  $\omega$ -azido-propane-sodium sulfonate.

5. A method for preventing anode sludge formation and for maintaining the purity of an acid copper plating bath which comprises the step of adding to said bath a compound selected from the group consisting of compounds having the following general structural formula:



and water soluble salts thereof, wherein R is a radical selected from the group consisting of lower saturated aliphatic hydrocarbon and aromatic hydrocarbon radicals, Z is an azido group and n is a whole number of at least one, said compound being added in an amount sufficient to prevent sludge formation.

6. A method for preventing anode sludge formation and for maintaining the purity of an acid copper plating bath which comprises the step of adding to said bath a compound selected from the group consisting of compounds having the following general structural formula:



and water soluble salts thereof, wherein R is a radical selected from the group consisting of lower saturated aliphatic hydrocarbon and aromatic hydrocarbon radicals, Z is an azido group and n is a whole number of at least one, said compound being added in an amount sufficient to prevent sludge formation.

7. A method for preventing anode sludge formation and for maintaining the purity of an acid copper plating bath and the brightness of electrodeposits obtained therefrom, which comprises the step of adding to said bath brightening agents selected from the group consisting of N-mono- and di-substituted dithiocarbamic acid alkyl ester- $\omega$ -sulfonic acids and their salts, and 1,3,5-triazine-2,4,6-tris-(mercapto-alkane-sulfonic acids), the amount of said brightening agent being sufficient to effect said brightening; and a compound selected from the group consisting of compounds having the following general structural formula:



and water soluble salts thereof, wherein R is a radical selected from the group consisting of lower saturated aliphatic hydrocarbon and aromatic hydrocarbon radicals, Z is an azido group and n is a whole number of at least one, said compound being added in an amount sufficient to prevent sludge formation.

8. A method for preventing anode sludge formation and for maintaining the purity of an acid copper plating bath comprising an aqueous acid solution of copper sulfate and at least 0.01 gm./liter of N,N-diethyl-dithiocarbamic acid ethyl ester- $\omega$ -sodium sulfonate as a brightening agent, the step of adding to said bath from 0.05 to 4.5 gm./liter  $\omega$ -azido-propane-sodium sulfonate.

#### References Cited in the file of this patent

#### UNITED STATES PATENTS

UNITED STATES PATENT OFFICE  
CERTIFICATION OF CORRECTION

Patent No. 2,950,235

August 23, 1960

Wennemar Strauss et al.

It is hereby certified that error appears in the above numbered patent requiring correction and that the said Letters Patent should read as corrected below.

Column 2, line 11, for "a.h./liter acid" read -- ampere-hours per liter of acid bath --; column 4, line 26, for "the group" read -- the group --.

Signed and sealed this 8th day of August 1961.

(SEAL)

Attest:

ERNEST W. SWIDER

Attesting Officer

DAVID L. LADD  
Commissioner of Patents